

## UNITED STATES PATENT OFFICE

GEORG BRUNHÜBNER, OF PFORZHEIM, GERMANY, ASSIGNOR TO ERNST GIDEON BEK, OF PFORZHEIM, GERMANY

## METHOD OF SOLDERING CHAINS, CHAINMESH OR THE LIKE

No Drawing. Application filed March 13, 1928, Serial No. 261,695, and in Germany March 17, 1927.

The uniting of the joints of chains, rings, chainmail or similar articles, has hitherto generally been done by soldering. In the operation of soldering, a flux, together with solder-metal or solder-metal alloys, are used which must be suited in each case to the metal to be soldered, in order that they may undergo a combination with the same.

For the reasons stated a great number of different solder-alloys are required, the preparation of which is difficult and complicated and requires great skill and causes great expense, and frequently such alloys cannot be successfully used.

15 It is generally recognized in this art that the oil used in the chain machine which sticks to the chains as a film on their surface prevents soldering. Such oil is also inside the joints. The solder core chain of such solid 20 wire chains must first be very carefully cleaned of all machine oil, dirt, fat and oxides, then they must be boiled in a flux, such as borax or the like, then the links must be broken, then the chain must be dipped in 25 a sticky solution, such as resin solved in alcohol, and then it must be rubbed with powdered graphite until it becomes covered with it all over. Then the chain is soldered in a soldering machine.

30 By the method forming the subject-matter of the present invention the foregoing and other objections to prior methods are obviated, as either no solder-metals are required to weld together the metals to be 35 united or cheap metals only need be used.

In the first case the means consist of non-metallic elementary substances or combinations of the same which have a reducing effect. Combinations of non-metallic 40 elementary substances may also be mixed with oxides. These means are admixed with liquid-media, for instance water, oil and the like, and applied at the soldering- or welding point.

45 In the other case non-metallic elementary substances or combinations of such substances with cheap powdered metallic addition, for instance zinc powder, brass-powder and the like, are mixed and liquid media 50 added to the mixture. The commonly used

metal-solders in the state of finest powder can be used when metals or metal-alloys are to be united the soldering of which is specially difficult, as for instance alloys containing aluminium or alloys containing platinum. 55 As combinations of non-metallic elementary substances, carbides and silicides, and as non-metallic elementary substances non-poisonous red phosphorus are, for instance, well adapted for use. A suitable oxide is for instance, silicic acid or ground quartz ( $SiO_2$ ).

60 The mixture of non-metallic elementary substances, for instance red phosphorus admixed with oil or water mentioned in the first case, are especially suitable for 8 carat gold and gold-plated metal; also for a gold-copper alloy or for a copper-zinc-alloy with gold plating or for tombac and copper.

65 A combination as in the second case, in which reducing elementary substances or the combinations of the same, the one with the other, with metal dust, for instance red phosphorus, oil, zinc-dust and a pure flux, like borax, are mixed together, is specially adapted for silver containing metals. 70

75 The uniting of the solder-joints is mainly obtained in the first case in that by reduction of the oxides existing on the joint-faces, a local softening is produced on and in the alloy for their union, as in welding. As a reducing like elementary substance, like phosphorus is very efficient as a small quantity of the same aids in the softening and uniting, especially when the heating is only short.

80 One feature of the invention is the use of finely powdered red phosphorus or its equivalents as an element of a soldering composition containing the other compounds also in a finely powdered state with or without additions of metallic powders. 85

85 The action of the phosphorus is manifold. By its burning in the soldering process the oil which sticks to the chain is burned up without residue, a great momentary and effective heat is produced, oxides occurring at and around the metal surfaces and joints are reduced, alloys are formed of the phosphorus and the metal of the goods and/or such metals which are admixed in a finely powdered state. The red phosphorus functions 90 95 300

as a far more intensive and powerful reducing agent than any flux hitherto employed. Hereby and by the heat produced in its burning all oily and fatty matter and oxides contained inside the joint are effectively removed.

The addition of oxygenous combinations, like ground quartz, and the presence of the same in the joint, exerts in many cases an action increasing the softening, as the phosphorus which is present liberates from the ground quartz the silicium, i. e. a second less volatile reduction means.

The mixtures mentioned in the second case of non-metallic elementary substances or combinations of such substances with powdered metallic-additions as zinc-dust or the like, with a suitable flux, have proved satisfactory, specially for silver and alpaca. In this case a stronger connection of the metal-joints to be united is obtained as the mixture of copper, brass, zinc or other metal-dust, and reducing non-metallic elementary substance, such as red phosphorus, causes a raising of the temperature to a particularly high degree at the soldering point and during the soldering moment, so as to effect the melting together of the materials in a manner substantially different from ordinary soldering and which welds the metals without compression. The metal-dust is, on the one hand, a heat transmission agent in the reducing-action of phosphorus on silver and alpaca and, on the other hand, it has a solder-forming action at the heating, as it forms together with metals from the material to be soldered a metal-mixture melting at a slightly lower temperature. For alpaca for instance zinc-dust alone as solder would not have a sufficiently great uniting effect, as during the heating portions of nickel, copper and zinc from the alpaca-alloy would not enter in substantial quantity into alloy with the zinc-dust.

With the aid of the non-metallic elementary substances mentioned, it is further possible to favorably influence the degree of hardness of the metal to be soldered or welded. When, for instance the material to be soldered or welded is already provided with soldering or welding means, and carborundum to which a little boric-acid may be added is then applied to the material and the so coated material then shaken in a suitable receptacle, the amount of solder or welding material in excess of that required is removed and there remains a mixture of carborundum and acid with a sufficient amount only of the welding means (phosphorus, oil) to soften the material to the degree desired. This carborundum-mixture is placed by more precise treatment in the region of the solder-point, in order to obtain that the hardness of the material of the article to be soldered or welded will be preserved,

and the softening produced only in the joint, in order to obtain the best possible metallic-combination for use in soldering and for durability of the article. The carborundum presents further the advantage that, for instance in connected single links, stiff-solderings are avoided. This substance exerts especially in a mixture with boric-acid, on the one hand, an oxidation-preventing effect upon the surface of the metals to be united, especially upon the joints, and prevents on the other hand, notwithstanding the presence of the boric-acid, stiff soldering by reason of the fact that at the temperature necessary for the welding it exerts a less softening effect than the phosphorus which is between the joints.

The viscous or thin liquid, pasty or merely moist soldering or welding means can be easily applied on the solder-points. In the manufacturing of chains or chainmail the solder-means can be applied by the same machine by which the chain or chainmail is produced. The goods to be soldered or welded might however be dipped into the pasty mixture, and the solder or welding means in excess then removed by scouring, the necessary quantity for the soldering action remaining at the solder point. In certain cases shaking with the slightly moistened solder and welding means is sufficient to remove the excess material.

After the dipping the addition means (water, oil or the like) in excess can be removed by centrifugal action, the material being subsequently scoured with dry powdered soldering or welding means.

The addition substance may also be applied by the chain- or chain mail-producing machine, prior to or during the treatment of the wire thereby.

A further advantage of this mixing of non-metallic elementary substances with powdered metallic additions results from the circumstance that on the wire ends or joints to be soldered or welded gaps are formed owing to the irregular feeding of the wires by the ring-forming machine or by wearing of machine elements. Such gaps cannot be bridged by non-metallic elementary substances alone, as they volatilize or burn under the action of heat.

The gaps may, however, be filled with powdered metallic additions prior to the soldering and the wire ends may be connected the one with the other at the soldering by a metallic filler in the gap.

Hitherto no soldering or welding process has become known which makes it possible to bridge gaps at the solder- and welding points. The two wire ends had either to be strongly pressed the one against the other or solder, inserted between the wire ends, had to be held between the wire ends by the pressure exerted on the same. It is difficult to

carry out this process even with a machine working with maximum precision.

All rings or chain-links having such gaps caused "miss soldering" to happen so frequently that only very short pieces of chain could be produced, which had to be joined subsequently by inserting and soldering intermediate links by hand, this being however rather expensive.

- 10 The use of liquids, like water, oil, liquid flux means and the like, serves to bring the non-metallic elementary substances, or metallic admixtures when they are used, into a pasty or viscous state. The solder substances 15 in this state flow into all fissures and gaps of the joint or solder point and stick on the metal to be soldered. It is unimportant in this connection whether the solder point presents a gap or whether the wire ends to be 20 soldered are strongly pressed the one against the other. In the latter case any excess quantity of solder substances will flow over the whole wire surface, after the material has been heated to soldering heat, thus preventing 25 ing a lumpy formation at the joint.

The adhering of the solder substance on the solder point can be obtained also by slightly moistening the solder material with liquid substances which are inherently sticky 30 or which make the composition sticky, like oil or liquid borax or water, and in applying subsequently at these points the dry solder substances which are made to stick on the soldering material by the liquid substances 35 which have previously been applied. Any solder substance which adheres to any other point than the solder may be removed by scouring.

From the foregoing it will be seen that 40 the sticking of solder substances on the solder point can be obtained also when the liquid and the solid non-metallic elementary substances or the admixture of metallic additions are applied separately. The solder substances 45 in either case adhere strongly so that any treatments subsequently necessary, for instance scouring to remove the solder in excess or covering to protect against oxidation, will not cause dropping off of the solder substance. The solder substance in the joint can 50 be removed only by washing off the solder material with benzine or the like.

As regards applying of the liquid substances to the material to be soldered, it may 55 be mentioned that they can be transmitted by rubbing the material between hands which have been moistened with these liquid substances. Mechanically this can be done by conducting the wire, during the treatment in 60 the chain making machine, in contact with an absorbent body impregnated with the liquid substance. Another manner consists in dipping the dry solder material into these liquid substances and in throwing off the 65 liquid substances by centrifugal action, so

that only a thin coating remains on the solder material.

It is to be understood that the oil may be incorporated or not with the soldering composition as put up for sale and use in accordance with this new method; that is to say that the composition may be put up for sale in a pasty or other suitably fluent condition and containing the oil as an ingredient, or that the composition may be put up for sale and use as a dry powder or in other suitable dry state and the oil added at the time of use to make it fluent, i. e., when a soldering operation is to be carried out. For economic reasons it is desirable to put up the composition in powder form and to add the oil at the time of use and, in soldering chain concatenations and the like, which are coated with oil the soldering operation is simplified and cheapened by rubbing the oil coated rings or links with the dry solder powder, by which means the necessity of cleaning the chain preparatory to soldering, as required heretofore, is obviated and the oil ingredient, in whole or in part, supplied. If, in such case, the oil on the chain is not in quantum sufficient the deficiency may be supplied by adding oil either to the chain or to the solder to be supplied thereto. This explanation is made in order that it may be understood that the claims are held to cover a method in which the solder composition used may be made and sold in either of the stated ways and in which the oil may be incorporated at any time before or at the time of use.

I claim:—

1. The method of soldering the ends of interconnected links or rings of chains or chain-mesh fabric, which consists in dipping a plurality of interconnected links into a fluid solder material, whereby the links are covered with the solder material and particles of the solder material caused to flow into the link gaps, removing from the links all solder material except that contained in the link gaps, and then subjecting the links to the action of heat to fuse the solder material in the gaps.

2. The method of soldering the ends of interconnected links or rings of chains or chain-mesh fabric, which consists in dipping a plurality of interconnected links into a fluent solder material containing oil and a reducing agent, whereby the links are covered with the solder material and particles of the solder material caused to flow into the link gaps, removing from the links all solder material except that contained in the link gaps, and then subjecting the links to the action of heat to fuse the solder material in the gaps and to raise the temperature at the soldering moment through the action of the reducing agent to a degree sufficient to effect the burning of the oil without residue.

3. The method of soldering the ends of interconnected links or rings of chains or chain-

- mesh fabric, which consists in dipping a plurality of interconnected links into a fluent solder material containing oil and a reducing agent so as to cause solder material to cover the surfaces of the links and to flow over the surfaces of the links and into the link gaps, removing from the links all solder material except that contained in the link gaps, and then subjecting the links to the action of heat to fuse the solder material in the gaps and to raise the temperature at the fusing moment to a degree to effect through the action of the reducing agent a burning of the oil without residue.
15. 4. The method of soldering the ends of interconnected links or rings of chains or chainmesh fabric, which consists in applying to the links and in the link gaps a carrier oil and a powdered chemical reducing substance in finely divided condition held in suspension by the oil and forming with the metal of the ring ends to be united a soldering material, removing from the links all soldering material except that contained in the link gaps, and then subjecting the links to the action of heat to fuse the soldering material in the link gaps and to effect through the action of the reducing agent a raising of temperature at the fusing moment to a degree to cause the burning of the oil without residue.
5. The method of soldering the ends of interconnected links or rings of chains or chainmesh fabric, which consists in applying to the interconnected links a fluent solder material containing oil and a powdered solder metallic substance and a reducing agent held in a carrier liquid so as to cause the solder material to flow over the surfaces of the links and into the link gaps, removing from the links all solder material except that contained in the link gaps, and then subjecting the links to the action of heat to fuse the solder material in the link gaps and through the action of said reducing agent to raise the temperature at the soldering moment to a degree to effect the burning of the oil without residue.
6. The method of soldering the ends of interconnected links or rings of chains or chainmesh fabric, which consists in applying to the link surfaces and into the link gaps a fluent material containing a carrier liquid and a powdered reducing agent of a character adapted to form with the metal of the ring ends a soldering composition, removing from the links all of such fluent material except that contained in the link gaps, and subjecting the links to the action of heat to effect a fusion of the solder composition and a raising of the temperature at the soldering moment by the action of the reducing agent to a degree to effect the elimination of the carrier liquid without residue.
7. The method of soldering the ends of interconnected links or rings of chains or chainmesh fabric, which consists in applying

ing between the ends of the links to be soldered a reducing substance held in a carrier vehicle and forming with the metal of the link ends a solder composition, and then heating the links to fuse such solder composition at a temperature chemically raised by the action of the reducing agent to effect the elimination of the carrier vehicle without residue.

8. The method of soldering the ends of interconnected links or rings of chains or chainmesh fabric, which consists in forming and flowing onto the surfaces of the links and into the link gaps a fluent solder composition containing a carrier oil, a powdered metallic solder substance, and red phosphorus, removing from the links all solder material except that contained in the link gaps, and then subjecting the links to the action of heat to fuse the solder material and to raise the fusing temperature by the action of the phosphorus to a degree to cause the oil to be burned without residue.

9. The method of soldering the ends of interconnected rings or links of a length of chain or chainmesh in the presence of oil, which consists in applying to the link gaps solder material and subjecting the links to the action of heat in the presence of a reducing agent acting to raise the temperature at the soldering points and during the soldering action to a degree sufficient to effect the fusion and union of the link ends and the burning of the oil to effect its elimination without residue.

10. The method of soldering the ends of interconnected rings or links of a length of chain or chainmesh, which consists in flowing a solder material in fluent form over the surfaces of the links and into the link gaps, and uniting by fusion the link ends and solder particles in the link gaps.

11. The method of soldering the ends of interconnected rings or links of a length of chain or chainmesh, which consists in flowing a solder material in fluent form over the surfaces of the links and into the link gaps, removing from the links the solder except those particles contained in the link gaps, and fusing the link ends and solder material in the link gaps.

12. The method of soldering the ends of interconnected links or rings of chains or chain mesh fabric, which consists in applying to the links and in the link gaps a composition comprising a liquid carrier vehicle and a powdered reducing substance held in suspension by said vehicle and forming with the metal of the link ends to be united a soldering material, and subjecting the links to the action of heat to fuse said soldering material and the link ends and to eliminate the carrier vehicle without residue.

13. The method of soldering the ends of interconnected links or rings of chains or

- chainmesh fabric, which consists in applying to the links and in the link gaps a liquid carrier vehicle and powdered red phosphorus held in suspension by the vehicle and adapted 5 under the action of heat to effect a fusion and connection of the metal of the link ends, and subjecting the ring ends to the action of heat to fuse and unite the same and to effect a burning of the carrier vehicle without residue.
- 10 14. The method of soldering the ends of interconnected links or rings of chains or chainmesh fabric, which consists in applying to the links and in the link gaps a carrier oil and a powdered reducing substance held in suspension by the oil and forming with the metal of the link ends to be united a soldering material, and then subjecting the rings to the action of heat to fuse said soldering material and to raise the temperature at the fusing moment to a degree to eliminate the carrier vehicle.
- 15 15. The method of soldering the ends of interconnected links or rings of chains or chainmesh fabric, which consists in applying to the links and in the link gaps a carrier oil and powdered red phosphorus held in suspension by the oil and forming with the metal of the ring ends to be united a soldering material, and then subjecting the links to the action of heat to fuse the soldering material in the gaps and to burn off the oil without residue.
- 20 16. The method of soldering the ends of interconnected links or rings of chains or chainmesh fabric, which consists in applying to the links and in the link gaps a liquid carrier vehicle and a non-metallic elementary reducing substance held in suspension there- 25 by and forming with the material of the ring ends to be united a soldering material, and subjecting the links to the action of heat to fuse the soldering material and to burn off the carrier vehicle without residue.
- 30 40 17. The method of soldering the ends of interconnected links or rings of chains or chainmesh fabric, which consists in applying to the links and in the link gaps a carrier oil and a powdered non-metallic ele- 45 mentary reducing substance held in suspen- 50 sion by the oil and forming with the metal of the ring ends to be united a soldering material, and then subjecting the links to the action of heat to fuse the soldering material and to burn off the oil without residue.
- 55 60 18. The method of soldering the ends of interconnected links or rings of chains or chainmesh fabric, which consists in applying to the links and in the link gaps a liquid carrier vehicle, a powdered non-metallic elementary reducing substance and a powdered oxygenous reducing substance held in suspen- 65 sion by said vehicle and forming with the metal of the ring ends to be united a soldering material, and subjecting
- the links to the action of heat to fuse the soldering material and burn off the carrier vehicle without residue.
- 70 19. The method of soldering the ends of interconnected links or rings of chains or chainmesh fabric, which consists in applying to the links and in the link gaps a carrier oil and a powdered non-metallic elementary reducing substance and a powdered oxygenous reducing substance, and subjecting the links to the action of heat to fuse said substance and the link ends and to burn off the oil without residue.
- 75 80 20. The method of soldering the ends of interconnected links or rings of chains or chainmesh fabric, which consists in applying to the links and in the link gaps a liquid carrier vehicle, a powdered non-metallic elementary reducing substance and a powdered oxygenous reducing substance held in suspen- 85 sion by the vehicle and forming with the metal of the ring ends to be united a soldering material, and then subjecting the links to the action of heat to fuse the soldering material and to eliminate the carrier vehicle.
- 90 95 21. The method of soldering the ends of interconnected links or rings of chains or chainmesh fabric, which consists in applying to the links and in the link gaps a carrier oil, a powdered non-metallic elementary reducing substance, a powdered oxygenous reducing substance, and a powdered metal held in suspension by the oil and forming with the metal of the ring ends to be united a soldering material, and then subjecting the links to the action of heat to fuse the soldering material and burn off the oil.
- 100 105 In testimony whereof I affix my signature.
- GEORG BRUNHÜBNER.
- 110
- 115
- 120
- 125
- 130